

# UNITED STATES PATENT OFFICE.

SHERBURNE B. HENNING, OF RHINELANDER, WISCONSIN, ASSIGNOR TO THE UNITED STATES OF AMERICA.

## GLUE AND PROCESS FOR MANUFACTURING THE SAME.

1,329,599.

Specification of Letters Patent.

Patented Feb. 3, 1920.

No Drawing.

Application filed April 22, 1919. Serial No. 291,973.

*To all whom it may concern:*

Be it known that I, SHERBURNE B. HENNING, a citizen of the United States, residing at Rhinelander, in the county of Oneida and 5 State of Wisconsin, have invented a new Glue and Processes for Manufacturing the Same, of which the following is a specification.

My invention relates to the manufacture 10 of glue and in particular, to that type of glue containing albumin, lime and ammonium hydroxid. The object of my invention is to produce a superior glue of this type and to disclose an improved process 15 for making this glue.

In preparing my glue I place in a suitable mixture 100 parts by weight of black soluble blood albumin. To this I add between 125 and 190 parts by weight of water, 20 not however, adding all the water at once but keeping out a small proportion of the water to be mixed with the lime used as will be hereinafter stated. The temperature of the blood albumin and the water should be 25 approximately 80 degrees Fahrenheit. After this mixture has soaked for approximately one hour, it is stirred slowly at first and then more rapidly. I then add, by stirring in, two to six parts by weight of ammonium 30 hydroxid of a specific gravity of 0.90. I then mix with from one to three parts by weight of lime, the water kept out of the quantity mixed with the blood albumin in order to produce a milk of lime. This milk 35 of lime is thoroughly mixed in and the entire mixture is stirred for approximately half an hour, after which the glue is ready for use.

Soaking the blood albumin in water at the 40 beginning of the process causes part of the albumin to dissolve in the water and softens the remainder. The addition of the ammonium hydroxid, however, dissolves much more of the albumin and leaves only a small 45 part of the albumin undissolved. In this way, the albumin is much more finely divided and comes into more intimate contact with the lime. The more intimate this contact, the greater the strength of the glue and 50 accordingly the addition of ammonium hydroxid produces a glue of greatly increased strength.

The addition of the ammonium hydroxid also retards the coagulation of the glue on 55 standing and, accordingly, the glue may be

used over a longer period after mixing. Further, the ammonium hydroxid reduces the surface tension of the liquid glue and thus facilitates penetration by the glue into the wood or other material to be glued. 60

I have found by experiment that, while lime adds strength to an albumin glue, there is a definite point after which the increase in the amount of lime will decrease the strength of the glue rather than increase it. 65 I have found that this optimum amount of lime is three per cent. by weight of the amount of albumin.

It is well known that sufficient water is required to dissolve and carry the albumin. 70 It is also well known that the strength of the joint depends on the proportion of solid material present. Balancing these two, I have found that the maximum strength is obtained when the weight of the water is 75 substantially  $1\frac{1}{2}$  times that of the albumin.

I also find that the use of a mixing temperature in excess of the coagulating temperature of albumin results in the coagulation of a considerable part of the albumin 80 and a consequent weakening of the glue. For that reason I maintain the temperature of the mixture well below the coagulating temperature and in fact maintain it below 85 degrees Fahrenheit. 85

In these several ways, I have improved the existing albumin glues. I have set forth the exact process and proportions preferred by me at present, but I realize that changes may be made and so far as these changes 90 fall within the scope of the appended claims, I deem them to be included in my invention. I also realize that other chemical materials may be substituted for one or more of these employed by me and in so far as such substitutions are obvious, I deem them included in my invention. 95

This application is a continuation in part of an application filed April 1, 1918, Serial No. 226,129. 100

What I claim is:

1. A glue comprising blood albumin, ammonium hydroxid, lime and water.
2. A glue comprising by weight substantially 1 part of blood albumin, .02 to .06 105 parts of ammonium hydroxid, lime and water.

3. A glue comprising by weight substantially 1 part of blood albumin, ammonium hydroxid, .01 to .03 parts of lime and water. 110

4. A glue comprising by weight substantially 1 part of blood albumin, ammonium hydroxid, lime and  $1\frac{1}{2}$  parts of water.
5. A glue comprising by weight substantially 1 part of blood albumin, .02 to .06 parts of ammonium hydroxid, .01 to .03 parts of lime and water.
6. The process of making an albumin glue which comprises mixing blood albumin, lime, ammonium hydroxid and water at a temperature below the coagulating temperature of blood albumin.
7. The process of making an albumin glue which comprises soaking blood albumin in water, adding ammonium hydroxid and then adding lime.
8. The process of making an albumin glue which comprises soaking blood albumin in water, thoroughly mixing in ammonium hydroxid, and thoroughly mixing in lime.
9. The process of making albumin glue which comprises soaking 1 part of blood albumin by weight in approximately  $1\frac{1}{2}$  parts of water, thoroughly mixing in .04 parts ammonium hydroxid and thoroughly mixing in .02 parts of lime.
10. The process of making an albumin glue which comprises soaking 1 part of blood albumin in water, mixing in approximately .04 parts ammonium hydroxid, and mixing in .02 parts lime.

In testimony whereof I affix hereunto my signature.

SHERBURNE B. HENNING.